

No. 734,743.

Patented July 28, 1903.

# UNITED STATES PATENT OFFICE.

ALFRED PAUL, OF MELROSE HIGHLANDS, MASSACHUSETTS.

## COMPOSITION OF MATTER FOR USE AS FUEL.

SPECIFICATION forming part of Letters Patent No. 734,743, dated July 28, 1903.

Application filed September 8, 1902, Serial No. 122,579. (No specimens.)

*To all whom it may concern:*

Be it known that I, ALFRED PAUL, a citizen of the United States, residing at No. 7 Union street, Melrose Highlands, in the county of Middlesex and State of Massachusetts, have invented a new and useful Composition of Matter to be Used as Fuel, of which the following is a specification.

My composition consists of the following ingredients, combined in the proportions stated, viz: coal-dust screenings or waste, fourteen to fifteen pounds; wood-sawdust, one to one and one-fourth pounds; resin, (ground,) one pound six ounces to one pound ten ounces; beer, (alcoholic, sour,) one-half gallon; molasses, four to eight ounces, first, my chief ingredient, consisting of coal-dust, screenings, or waste, the refuse deposit of anthracite and bituminous coal; the second ingredient, (wood-sawdust,) sawdust from pine, spruce, cypress, chestnut, birch, ash, elm, oak, white-wood, hemlock, hickory, maple, or mahogany; the third ingredient, (resin,) common pine-resin, ground; the fourth ingredient, (beer, alcoholic, sour,) this ingredient to consist of either ale, porter, or lager when it becomes

a refuse or sour, said ingredients made from malt and hops; the fifth ingredient, (molasses,) this ingredient to consist of the low-grade sugar-molasses, the above ingredients to be thoroughly mixed in the proportion already described, these ingredients to be thoroughly mixed. The composition is then pressed into forms, baked or dried to a hard solid body, the forms to be square, oblong, 35 or any convenient shape suitable for kitchen-range, fireplace, stove, heater, furnace, or engine-boiler.

I hereby claim and desire to secure by Letters Patent of the United States—

The composition of ingredients herein described, consisting of coal-dust, screenings or waste, wood-sawdust, resin, sour beer (alcoholic) and molasses, mixed together, to form a fuel from coal-dust, substantially as 45 described and for the purpose specified.

In testimony whereof I have affixed my signature in presence of two witnesses.

ALFRED PAUL.

Witnesses:

GEORGE HENRY KIRMES,  
GEORGE WALLACE BURKE.